

Oct. 7, 1924.

1,510,747

H. C. PRIVETT

INNER TUBE

Filed March 1, 1922

*Fig. 1.*



*Fig. 2.*



*Fig. 3.*



*Fig. 4.*



Executor:  
H. C. Privett.  
by Hazard E. Miller  
Atty.

Patented Oct. 7, 1924.

1,510,747

# UNITED STATES PATENT OFFICE.

HENRY C. PRIVETT, OF LOS ANGELES, CALIFORNIA, ASSIGNOR OF ONE-HALF TO CHARLES ROBERT PRIVETT AND ONE-FOURTH TO HOLLIS F. PRIVETT, BOTH OF LONG BEACH, CALIFORNIA.

## INNER TUBE.

Application filed March 1, 1922. Serial No. 540,163.

To all whom it may concern:

Be it known that I, HENRY C. PRIVETT, a citizen of the United States, residing at Los Angeles, in the county of Los Angeles and State of California, have invented new and useful Improvements in Inner Tubes, of which the following is a specification.

My invention relates to inner tubes for pneumatic tires, and particularly to that type of inner tube in which a reinforcing strip is embedded in the thickened tread portion for preventing undue transverse expansion of the outer tread surface so as to effect a compression of the inner tread surface sufficient to provide self-sealing means for punctures.

In tubes of the above type, the reinforcing strip is formed of a fibre, generally canvas, which is capable of longitudinal stretching only, the result being that in practice the stresses exerted transversely of the tube when the latter is inflated act to tear away the tube from the longitudinal edges of the reinforcing strip, thus preventing the strip from performing the function for which it is intended.

It is the purpose of my invention to provide a reinforcing strip which is so formed that when incorporated in the tread portion of a tube it becomes an integral part, and while successfully retaining the outer surface from undue expansion, it eliminates all possibility of its edges becoming disengaged or tearing away from the rubber.

In carrying out my invention I form the reinforcing strip of rubber in which is embedded textile fibres such as cotton fibres. The fibres are disposed transversely of the strip and substantially in two lengths, with the longer fibres disposed between the marginal edges of the strip and the short fibres at the marginal edges. This arrangement of fibres allows of the necessary longitudinal stretching of the strip to permit of its conforming to the contour of the tube, but prevents transverse stretching of the strip in the area covered by such fibres. These long fibres terminate at the marginal edges of the strip and in so doing permit of a transverse stretching of the marginal edges which, in conjunction with the longitudinal stretching permitted as a result of the transverse arrangement of the short fibres, positively

prevents the disengagement or tearing away of the longitudinal edges of the reinforcing strip from the inner tube thus insuring of the strip performing its function indefinitely.

In the accompanying drawings,

Figure 1 is a view showing a portion of a reinforcing strip constructed in accordance with my invention.

Fig. 2 is a sectional view of an inner tube having incorporated therein the reinforcing strip shown in Fig. 1, the tube being shown in the form it assumes prior to its reversal or to the position shown in Fig. 3.

Fig. 3 is a fragmentary perspective sectional view of the tube shown in Fig. 2 and in the position in which it is applied to a tire casing.

Fig. 4 is a sectional view of a tire casing with the tube shown in Fig. 3 in inflated position therein.

Referring specifically to the drawings and particularly to Fig. 1, the reinforcing strip is designated at S and is shown as comprised of cotton waste and rubber of the same character as that of which the tube is formed. In forming the reinforcing strip, a relatively large sheet composed of cotton waste and rubber is first formed by passing the waste and rubber through rollers (not shown) which serve to draw the cotton fibres in the same general direction within the sheet. This sheet of material is cut transversely of its length into strips of suitable width so that the fibres contained within each strip are disposed transversely of its length. By forming the strips in this manner relatively long lengths of fibres are disposed along the longitudinal axis of each strip, while at the marginal edges of the strip are located relatively short fibres. As previously explained, the long fibres serve to prevent transverse stretching of the strip, while the short fibres allow of a transverse stretching of the marginal edges of the strip. The arrangement of the long and short fibres within the strip is clearly illustrated in Fig. 1.

When forming the inner tube shown in Fig. 2, the thickened tread portion 15 thereof is vulcanized with the reinforcing strip S in the position shown, so that the rubber of the strip co-operates with the rubber of the tread portion to form a homogeneous mass which securely retains the strip in

proper position within the tread portion and thus insures of the fibres performing the functions for which they are designed. As a result of the arrangement of the fibres, the 5 reinforcing strip is now free to stretch longitudinally, but transversely along its marginal edges only, so that when the tube is inflated and thus subjected to transverse stresses, the reinforcing strip will give at 10 its edges under the expanding action of the tube to prevent disengagement or tearing away of the edges of the strip from the rubber of the tube. It is to be understood, however, that the long fibres continue to prevent 15 any appreciable stretching of the major portion of the strip so that the latter continues to prevent stretching of the outer tread surface of the tube when in applied position within a tire casing as shown in 20 Fig. 4.

What I claim is:

1. In combination, an inner tube having a thickened tread portion, and a reinforcing

sheet embedded within the tread portion and comprising a fibrous material completely 25 impregnated with rubber and with the latter vulcanized with the rubber of the tread portion for the purpose described.

2. A reinforcing strip for the tread portion of inner tubes comprising an elastic 30 material, short and long inelastic members embedded within the material and arranged transversely of the strip, the long members being arranged between the marginal edges of the strip, and the short members at the 35 marginal edges.

3. An inner tube for an automobile tire comprising a ring of rubber having natural fibers embedded in the tread thereof, said natural fibers being arranged in interlacing 40 relationship with a preferred tendency to lie across the tread of the tire.

In testimony whereof I have signed my name to this specification.

HENRY C. PRIVETT.